

# UNITED STATES PATENT OFFICE.

EUGÈNE BARON, OF PARIS, FRANCE.

## DECORATIVE FABRIC.

SPECIFICATION forming part of Letters Patent No. 287,495, dated October 30, 1883.

Application filed June 9, 1883. (No specimens.)

*To all whom it may concern:*

Be it known that I, EUGÈNE BARON, of the city of Paris, France, have invented a new kind of Decorative Fabrics, of which the following is a full, clear, and exact description.

This invention consists in the manufacture of a new kind of decorative fabrics.

In order to produce my fabric, I deposit upon thread, cotton, woolen, or other fabrics, or upon leather, linoleum, and the like, crystallizations of alloys of bismuth, antimony, and tin in various proportions, employing for this purpose chemical agents and appropriate apparatus, or effecting it by means of electro-metallurgy, or any of the known means of electricity. I brighten the crystallized layers by means of acidulated baths, and I obtain crystallized surfaces with various effects. I then make a suitable design on stone or zinc, and by any means employed in the trade for printing. I submit my fabrics or other matters prepared as above-described to this printing-plate, employing suitable printing colors, velvet powder, mica powder, &c., and the metallic bronzes. The parts of the design that

are not covered with the printing color or substance stand out from the opaque ground and appear in all their brilliancy. I finally place upon the crystallized threads, by hand or otherwise, transparent colors—such as spirit-varnishes, tinted oil-varnishes, or other transparent colors.

Applied to linoleum my invention is of especial value.

I do not claim attaching metal foil to fabrics. In such foil the particles of the metal adhere together, while my crystalline deposits adhere only to the fabric, and therefore do not interfere with the flexibility of the fabric, nor with the durability of the ornamentation.

I claim—

The process herein described of ornamenting fabrics, which consists in depositing upon them crystallized metallic alloys, and then partly covering the crystallized surfaces by printing, substantially as specified.

EUGÈNE BARON.

Witnesses:

ROBT. M. HOOPER,

JEAN BAPTISTE ROLLAND.

It is hereby certified that in Letters Patent No. 287,495, granted October 30, 1883, upon the application of Eugène Barou, of Paris, France, for an improvement in "Decorative Fabrics," the name of the patentee was incorrectly written and printed "Eugène Baron," instead of *Eugène Barou*; and that the proper correction has been made in the files and records pertaining to the case in the Patent Office, and should be read in the patent to make it conform thereto.

Signed, countersigned, and sealed this 25th day of December, A. D. 1883.

[SEAL.]

M. L. JOSLYN,  
*Acting Secretary of the Interior.*

Countersigned:

BENJ. BUTTERWORTH,  
*Commissioner of Patents.*